

## UNITED STATES PATENT OFFICE

HERBERT PLATT, OF CUMBERLAND, MARYLAND, ASSIGNOR TO CELANESE CORPORATION OF AMERICA, A CORPORATION OF DELAWARE

## SIZING OF DYED YARN

No Drawing.

Application filed July 13, 1928. Serial No. 292,605.

This invention relates to the sizing of yarn that has been previously dyed, and relates more particularly to the sizing of yarn containing organic derivatives of cellulose, which have been dyed with a dye that is normally insoluble in water.

An object of my invention is to dye yarns of all kinds, but particularly yarns made of or containing organic derivatives of cellulose such as cellulose acetate, in such a manner that the dyed yarn suffers but little change in color after the sizing compound is removed.

The sizing of dyed yarn, and particularly 15 yarn containing organic derivatives of cellulose that have been dyed with certain water insoluble dyes that are solubilized by means of a dispersing agent, has heretofore presented serious difficulty. If an attempt is made to 20 size such dyed yarn by the ordinary methods, it is found that the color tends to bleed both into the sizing bath and also into the bath that is used for removing the size after the required textile operation. Moreover, the textile 25 product thus formed is often dull in color and has other undesirable characteristics.

In accordance with my invention, I treat a 30 yarn containing organic derivatives of cellulose, that has been dyed in any desired manner, with a sizing composition containing glue or gelatin that is substantially neutral and at a suitable temperature.

The yarn to be treated in accordance with 35 my invention may contain any suitable organic derivatives of cellulose such as organic esters of cellulose or cellulose ethers. Examples of organic esters of cellulose are cellulose acetate, cellulose formate, cellulose propionate and cellulose butyrate. Examples of cellulose ethers are ethyl cellulose, methyl cellulose and benzyl cellulose.

The yarn may consist wholly of one or 40 more of these organic derivatives of cellulose or it may be a mixed yarn containing fibres of these organic derivatives of cellulose and

fibres of other materials such as cotton, silk or wool. Examples of such mixed yarns are mixed cellulose acetate and cotton and mixed cellulose acetate and wool.

The yarn to be sized may be dyed by any 50 suitable dye. However, this invention is particularly applicable to yarns that have been dyed with water insoluble dyes which have been solubilized by a dispersing agent. An example of a series of such dyes, are the 55 anthraquinone vat dyes in the unreduced state dispersed in aqueous suspension by means of dispersing agents, such as sulpho fatty acids of which sulpho ricinoleic acid is an example. The yarn may be dyed by a single dye or by a mixture of dyes to obtain 60 the desired color.

The sizing bath contains glue or gelatin and is substantially neutral. It may be slightly alkaline but it is preferable that it 65 should not have an acidic reaction. Generally a sizing bath having a pH value of 7 to 7.5 is preferred in my process. The temperature of the sizing bath should preferably be from 60° to 80° C. I have found that a temperature of 70° C. produces the best results.

After the yarn has been sized in the bath 70 it may then be woven or knitted into a fabric or subjected to any other desired textile operation. The material is then desized by submersion in or by other treatment with water at a temperature of 50° to 70° C. but preferably 60° C. The dye bleeds but little and the textile material thus produced is found to have a color that is substantially as bright as 75 the dyed material before it has been sized.

In order further to illustrate my invention 80 the following specific example is given but my invention is not limited thereto.

## Example

A yarn consisting wholly of cellulose acetate is dyed with any suitable dye, such as 85 1,4 dimethyldiamino anthraquinone or 2,4 dinitro 4' amino diphenylamine dispersed in 90

aqueous suspensions by means of sulfo ricinoleic acid, or any other dyes such as setacyl or the so called direct or dispersol dyes.

5 The dyed yarn is then sized with a sizing composition at 70° C., such composition being made up as follows:

|                 |      |        |
|-----------------|------|--------|
| Gelatin         | 9    | pounds |
| Glycerine       | 2    | pounds |
| Castor oil      | 1.5  | pounds |
| Sodium benzoate | 0.25 | ounce  |
| Water           | 260  | pounds |

This bath is caused to have a pH value of 15 7.0 to 7.5 by the addition of 1 lb. 5 ozs. to 1 lb. 6 ozs. of sodium carbonate. Because of the pH value of this sizing composition, change of shade of the dyed yarn is prevented, with practically no bleeding of the 20 dye.

It is to be understood that the foregoing detailed description is given merely by way of illustration and that many variations may be made therein without departing from the 25 spirit of this invention.

Having described my invention, what I claim and desire to secure by Letters Patent is:

1. Method of sizing yarn containing organic derivatives of cellulose, which yarn has previously been dyed with a water insoluble dye that is dispersed in an aqueous liquid by means of a sulfo-fatty acid, comprising treating the same with a sizing bath 30 containing gelatin which bath has a pH value of substantially 7 to 7.5, at a temperature of 60° to 80°.

2. Method of sizing yarn containing cellulose acetate, which yarn has previously been dyed with a water insoluble dye that is dispersed in an aqueous liquid by means of a sulfo-fatty acid, comprising treating the same with a sizing bath containing gelatin which bath has a pH value of substantially 40 45 7 to 7.5, at a temperature of 60° to 80° C.

3. Method of sizing yarn containing cellulose acetate, which yarn has been previously dyed with an anthraquinone vat dye in the unreduced state that is dispersed in an aqueous liquid by means of a sulfo ricinoleic acid comprising treating the same with a sizing bath containing a gelatin which bath has a pH value of substantially 7 to 7.5, at a temperature of substantially 50 55 70°.

55 In testimony whereof, I have hereunto subscribed my name.

HERBERT PLATT.